

# UNITED STATES PATENT OFFICE.

GEORGE A. SWEETMAN, OF BICKFORD, OKLAHOMA.

## TANNING-OOZE.

No. 901,564.

Specification of Letters Patent.

Patented Oct. 20, 1908.

Application filed February 24, 1908. Serial No. 417,540.

*To all whom it may concern:*

Be it known that I, GEORGE A. SWEETMAN, a citizen of the United States, residing at Bickford, in the county of Blaine and State of Oklahoma, have invented a new and useful Tanning-Ooze, of which the following is a specification.

This invention relates to tanning oozes.

The object of the invention is to provide an ooze which shall be adapted, in a ready, rapid and economical manner, to tan hides and pelts, and the ingredients of which shall be readily procurable in almost any locality, and the preparation of ooze requiring no especial machinery or apparatus for the purpose.

With the above and other objects in view, as will appear as the nature of the invention is better understood, the same consists in the novel tanning ooze hereinafter described and claimed.

In carrying the invention into effect, there is taken of soft water ten gallons, Bengal catechu, one quarter of a pound, septfoil root (*Potentilla tormentilla*) three pounds, aleppo galls, one-half pound, ground hops, one quarter of a pound, and powdered gum senegal, one fourth ounce. All of the ingredients, with the exception of the gum senegal, are placed in the water, and the latter is brought to and retained at the boiling point

for one hour, or more. It is then allowed to cool and the gum senegal is then added and thoroughly stirred into the ooze.

In the use of the bath, the hides or pelts are allowed to remain therein from two to seventeen days, according to the character of the hide or pelt, and when the necessary period has elapsed, the article will be found to have been thoroughly tanned. The usual washing and oiling down may be employed if found necessary or desirable.

I claim:

1. The herein described tanning bath consisting of soft water, Bengal catechu, septfoil root, aleppo galls, ground hops, and powdered gum senegal, substantially in the proportions specified.

2. The herein described tanning bath consisting of soft water, ten gallons; Bengal catechu, one-fourth pound; septfoil root, three pounds; aleppo galls, one-half pound; ground hops, one-fourth pound; and powdered gum senegal, one-fourth ounce.

In testimony that I claim the foregoing as my own, I have hereto affixed my signature in the presence of two witnesses.

GEORGE A. SWEETMAN.

Witnesses:

W. A. HOUGH,  
R. I. TEMPLE.